

## UNITED STATES PATENT OFFICE

1,981,643

## VISCOSE SPINNING SOLUTION

Rudolph S. Bley, Elizabethton, Tenn., assignor to  
North American Rayon Corporation, New York,  
N. Y., a corporation of Delaware

No Drawing. Application December 29, 1933,  
Serial No. 704,514

4 Claims. (Cl. 106—40)

The present invention relates to a process of producing viscose filaments having light-reflecting properties differing from those produced in a conventional manner.

One object of my invention is to incorporate into viscose spinning solutions a compound which will produce an effect upon the light-reflecting qualities of the finished filaments such that they will appear to be of a duller lustre than ordinary filaments.

Another object of my present invention is to produce a viscose spinning solution which will yield filaments possessing a sheen lustre resembling that of real silk.

A third object of my invention is to incorporate a mono-thiocarbonic acid ester, a tri-thiocarbonic acid ester or a metallic salt of such esters into a viscose spinning solution to produce dull lustre filaments.

A fourth object of my invention is to produce a new delustering agent for viscose filaments, said agent comprising mono-thiocarbonic acid esters or tri-thiocarbonic acid esters of aliphatic or aromatic alcohols and of other organic compounds having reactive OH groups.

Other objects of my invention will become apparent to those skilled in the art from a study of the following specification.

When cellulose is impregnated with a mercerizing solution of caustic soda, and carbon bisulphide is subsequently added thereto, a water-soluble sodium salt of cellulose xanthogenate is produced. This salt is generally called "viscose", and it may readily be decomposed with

the formation of gelatinized cellulose. Theoretically, during the viscose reaction, sodium cellulose xanthogenate is formed in accordance with the following equations:



45 The viscose solution spontaneously decomposes on standing with the liberation of gelatinized cellulose. In "ripening", there is first observed a progressive decrease in viscosity, due to the depolymerizing action of the excessive alkali, and then an increase in viscosity takes place, since coagulation gradually sets in. This viscose solution, after proper ripening, is spun or extruded in the form of fine filaments into a setting bath comprising acids and sulphates.

55 I am well aware that starch xanthogenates

have, heretofore, been used for the manufacture of filaments, films and the like, and that U. S. Patent No. 1,937,110 of November 28, 1933 to Elssner discloses the addition of salts of dithiocarbonic acid-o-isobutyl ester, but I verily believe myself to be the first inventor to propose the addition of mono-thiocarbonic acid esters, tri-thiocarbonic acid esters and/or metallic salts of such esters as delustering agents for viscose filaments. Aliphatic alcohols, such as methyl, 60 ethyl, propyl, butyl alcohol, etc., i. e. alcohols having the structure  $C_nH_{2n+1}$ , aromatic alcohols and other organic compounds, such as starches, having reactive OH groups, may be treated with mono- or tri-thiocarbonic acids to yield corresponding esters which are adapted to be mixed singly or in combination with viscose spinning solutions in order to produce the aforesaid effect. I have, furthermore, found that thiocarbonic acid esters, set forth above, may be treated with metal salts to produce soluble or insoluble compounds suitable as delustering agents, the solubility of the reaction product depending upon the characteristics of the specification introduced.

50 Mono-thiocarbonic acids, thiocarbonic acids and tri-thiocarbonic acids may be caused to react with aliphatic alcohols, aromatic alcohols and other organic compounds having reactive OH groups to form esters. The following table depicts a series of esters capable of modifying viscose silk, but it is to be noted that my invention is not limited to these compounds which are merely given as examples.

|                                                                     | Boiling point |
|---------------------------------------------------------------------|---------------|
| Thio-ethyl carbonic ethyl ester                                     | 156° C.       |
| Thion-carbonic acid ethyl ester                                     | 161° C.       |
| Tri-thiocarbonic methyl ester                                       | 205° C.       |
| Tri-thiocarbonic ethyl ester                                        | 240° C.       |
| Mono-thiocarbonic starch ester, tri-thiocarbonic starch ester, etc. | 95            |

These esters may be treated with metals, for example, sodium, potassium, calcium, barium, strontium, etc., or with equivalent amounts of 100 metallic salts to produce metallic derivatives of mono- or tri-thiocarbonic acid esters, respectively. The calcium salt, for example, of mono-thiocarbonic-o-isobutyl ester may be formed during the mercerization step, and it may be added to 105 the viscose solution prior to spinning. Besides calcium, other metals, such as sodium, barium, strontium, etc., may be introduced to form delustering agents for viscose in combination with thiocarbonic acid starch esters. Depending upon 110

the metal introduced, soluble or insoluble metal salts are formed in the viscose filaments. The nature of the alkyl group and the residual organic groups, respectively, governs the formation of 5 organic compounds which, upon evaporation, will have the effect of reflecting light in such a manner that filaments of very dull lustre are produced. The amounts of the new delustering agents to be added to viscose may be varied with- 10 in wide limits, although I have found that an admixture of about 5 to 10% will produce very satisfactory results.

*Example*

15 To a 1000 liter batch of a viscose spinning solution, containing about 7.5% cellulose and 6.8% sodium hydroxide, are added 6 kilograms of calcium mono-thiocarbonic-o-isobutyl ester. The mixture is thoroughly stirred and spun under 20 conventional conditions.

I wish to point out that the compounds, as well as their quantities to be admixed to viscose spinning solutions set forth above, are merely

25

30

35

40

45

50

55

60

65

70

75

illustrative and, thus, may be varied without departing from the spirit and scope of my invention. No limitation should be imposed upon my invention except as indicated in the appended claims.

80 I claim:

1. A spinning solution for the manufacture of soft-lustre products comprising a viscose solution and an aliphatic ester of a mono-thiocarbonic acid uniformly dispersed therein.

85 2. A spinning solution for the manufacture of soft-lustre products comprising a viscose solution and a starch ester of a mono-thiocarbonic acid.

90 3. A spinning solution for the manufacture of soft-lustre products comprising a viscose solution and a metal salt of an aliphatic ester of a mono-thiocarbonic acid.

95 4. A spinning solution for the manufacture of soft-lustre products comprising a viscose solution and a mono-thiocarbonic-o-isobutyl-ester.

RUDOLPH S. BLEY.

100

105

110

115

120

125

130

135

140

145

150